

## UNITED STATES PATENT OFFICE

LEO B. KIMBALL, OF NAUGATUCK, CONNECTICUT, ASSIGNOR TO FUEL DEVELOPMENT CORPORATION, A CORPORATION OF DELAWARE

## FUEL

No Drawing.

Application filed January 31, 1931. Serial No. 512,747.

This invention relates to liquid hydrocarbons, commonly used as fuels in internal combustion engines of the explosive type, particularly in automobile engines and in similar engines for other power purposes.

The object of my invention is to produce a liquid fuel which shall have suitable vaporization characteristics and can be used in high compression engines of the above mentioned type and which will also reduce the tendency, during combustion, to produce preignition, detonation or knocking.

It has been appreciated by various investigators in the art of hydrocarbon fuels for engines of the explosive type that aniline when added to a commercial fuel such as gasoline with a blending agent such as butanol, is efficacious in reducing detonation but its use in gasoline and similar fuels is accompanied by various disadvantages which it has been thought to be practically impossible to eliminate.

One of these disadvantages is that when aniline is mixed with gasoline or similar hydrocarbon fuel, the aniline has crystallized out and becomes separated from the gasoline at temperatures in the vicinity of 10° above zero Fahrenheit. Various attempts have been made to prevent this crystallization of the aniline at low temperatures and some have been more or less successful by using as an additional ingredient, some more expensive fluid or liquid so that the homogeneity of the fuel is increased even at quite reduced temperatures.

These considerations become of great importance when gasoline is used in airplanes which often, even in summer, reach high altitudes where the temperature may fall to from 25° to 50° below zero, Fahrenheit. A large proportion of benzol is usually incorporated with gasoline when the fuel is to be used at such low temperatures, to produce the necessary anti-knock characteristics.

I am familiar with the results of research of prior experimenters and patentees along these lines, but am not aware that any of them have attained the results and perfection of liquid hydrocarbons as fuels for internal combustion engines that I have at-

tained by the combination of ingredients described below.

I have attempted to attain two more important objects in the researches which I have carried out along the lines above indicated. The first is to produce such a mixture of a hydrocarbon fuel and aniline that no crystals will be separated from the fuel even when the temperature is reduced to as low as 40° F. below zero.

This result is attained mainly by adding to a mixture of aniline, butanol and an hydrocarbon fuel, such as gasoline, a small percentage (usually less than 1%) of ethyl alcohol of low moisture content. The second result which I have attempted to obtain and have attained, is the retention of aniline and alcohol together in solution in gasoline so that the same are not affected by the presence of water which may thereafter become mixed with the gasoline owing to condensation and of moist atmosphere or other sources of moisture. This latter result is brought about by the fact that a small quantity of ethyl alcohol so combines with the aniline and butanol that the latter ingredients are not affected by the subsequent addition of moisture, and the aniline is therefore prevented from being crystallized even at such low temperatures as minus 40° F. Another advantage in using ethyl alcohol for this purpose is that the alcohol itself aids in reducing the tendency to preignition or knocking.

Ordinarily it is desirable to use from 1% to 3% of aniline with one-tenth of one per cent. to one per cent. of butanol in gasoline used for the motor fuel. The amount of ethyl alcohol to cause the aniline to remain in solution should range from two-tenths or three-tenths of one per cent. up to three per cent. or slightly more, depending upon the amount of aniline introduced and the lower points of temperature to which the fuel may be subjected.

It will, of course, be appreciated that the higher the compression during the compression stroke of an automobile engine, the larger the amount of aniline will be necessary to eliminate the detonation or knock.

Further advantages resulting from the

use of my improved mixtures as fuels for internal combustion engines, arise from the fact that the temperatures of combustion are reduced to a lower point than can be obtained by the more common and somewhat inferior fuels in general use.

It has been found in the use of many commercial fuels in engines for aeroplanes that such fuels heat the cylinder walls, the piston 10 and the valves to such an extent that they can only be driven for a short time without substantial loss of power and subsequent damage to the engine. The use of my improved fuel has been found to reduce the combustion temperatures very materially and to a point where they are not detrimental to the working parts 15 of an internal combustion engine. Often, the effects of detonation in an engine, when they exist, are indicated largely by high cylinder head temperatures. It has been found that during the wide open throttle operations 20 of aircraft engines, certain fuels cause a marked rise in cylinder head temperatures which results in considerable damage to the valves and valve seats and in some cases the blowing in of the piston heads.

A new scale of anti-knock ratings, recently adopted by automotive engineers, is based on a comparison of any particular fuel with a 30 mixture of iso-octane in normal heptane, the result being that a certain percentage of iso-octane can be introduced into the heptane to produce the same amount of detonation under similar conditions as is produced by the fuel being compared therewith. In other words, the percentage of iso-octane used in a mixture with heptane, designates the anti-knock rating. Since normal heptane is considerably worse from a knock standpoint, 40 than any of our common, modern fuels, and since iso-octane is better than any known fuel, these are taken as the ultimate zero and 100% values. Thus, mixtures of the two can be made which will duplicate any of the 45 present commonly used fuels. Present automobile gasoline ranges from a 50 octane number for very poor grades, to 64 for an average grade. In aircraft work best results are obtained with fuels having octane numbers approaching 100.

In the case of aniline mixtures as described in this application, much advantage results from the fact that a neutral oil is used which contains no metallic element and therefore it can be added in sufficient quantities without injury to the engine and without forming scaly deposits on the exhaust valves and other parts, such as may result from the use of fluids containing metallic elements. It is also 50 practically non-poisonous and does not require special precautions to prevent serious injury to operatives. The mixtures may be used at high altitudes where the atmospheric temperatures drop to low points. Furthermore, it has been found that the use of aniline

mixtures as stated in connection with the fuels of this invention, produces an anti-knock value in the vicinity of 3.5 octane numbers for each percent of the aniline mixture added to the fuel and the octane number may 70 be raised to 100 or more. Thus, it is apparent that the anti-knock value of a fuel may be definitely controlled and the heating action upon the parts of an internal combustion engine may be reduced to the desired 75 point for best efficiency under any conditions which may apply to an aircraft or automobile engine.

Some hydrocarbon fuels which work well at low temperatures of combustion will not 80 work at high temperatures because of the heating effect produced, and on the other hand, fuels which work at high temperatures, such as in aeroplane engines, will not work well at lower temperatures of combustion, 85 such as in automobile engines. Fuels which are made in accordance with the invention described in this application can be made to work well at either high or low temperatures of combustion, according to the amount of 90 aniline and other ingredients added. In other words, the addition of aniline, together with the other ingredients stated, results in the elimination of the effects of bad constituents of poor gasoline, such as the abnormal production of heat, as well as knocking, while at the same time the addition of such ingredients reduces the heating effect and raises the octane number. In fact, these effects may 95 be controlled and the desired octane number 100 may be produced even in the poorer grades of fuel.

It will be obvious to one skilled in the art that the proportions of aniline, butanol and ethyl alcohol that are used will be more or less dependent upon the constituents of the fuel used. I, therefore, do not wish to be limited to any specific proportions thereof, although the same should be substantially within the range of percentages above mentioned for best results.

What I claim as new and desire to protect by Letters Patent is:—

In a motor fuel for internal combustion engines of the explosive type comprising, an 115 hydrocarbon such as gasoline, the improvement which comprises the combination therewith of small percentages of aniline, butanol, and ethyl alcohol to prevent crystallization 120 of the aniline at low temperatures and which combination prevents the separation of the ingredients in the presence of moisture condensed therein or otherwise introduced.

Signed this 30th day of January, 1931.

LEO B. KIMBALL.

121

130